

# United States Patent Office.

JOHN STENHOUSE, OF 17 RODNEY STREET, PENTONVILLE, LONDON, ENGLAND, AS-SIGNOR TO ARTHUR CHENEY AND ALONZO MILLIKEN, OF BOSTON, MASSACHUSETTS.

*Letters Patent No. 97,983, dated December 14, 1869; patented in England, January 8, 1862.*

## IMPROVEMENT IN WATER-PROOFING FABRICS.

The Schedule referred to in these Letters Patent and making part of the same.

*To all whom it may concern:*

Be it known that I, JOHN STENHOUSE, of 17 Rodney street, Pentonville, London, England, chemist, have invented certain new and useful Improvements in Rendering certain Substances less Pervious to Air and Liquids, and also less liable to decay; and I hereby declare the following to be a full, clear, and exact description of the same.

My said invention relates to the use of the substance called paraffine, in a solid state, for the purpose of rendering various substances less pervious to air and liquids.

The substances to which I propose to apply the paraffine, are wood, leather, paper, and textile fabrics composed of cotton, linen, wool, or silk; and my method of applying the paraffine to such substances consists in coating or impregnating them therewith.

One way in which I treat leather and textile fabrics is as follows:

I take a plate of iron, or other metal, the upper surface of which is quite clean, and this I heat to a temperature of from 130° to 250° Fahrenheit, or even higher, if desirable, either by placing it over a suitable furnace, or by means of low or high-pressure steam, or a metallic or other bath.

On this plate I stretch out the cloth or leather which I wish to coat or impregnate, and hold it tight and flat, by means of a frame, or some other suitable arrangement. When it has become sufficiently warm to soften or melt the paraffine easily, I then rub over it, on the wrong side of the cloth, a flat rectangular block of solid paraffine, with the hand or otherwise, so as to coat its surface as evenly as possible. The cloth is then strongly compressed, by means of a hot flat-iron, or hot rollers, or other suitable arrangement, in order to distribute the paraffine more equally among the fibres.

When the coating or impregnation of the fibres is completed, it is taken off and allowed to cool.

Sometimes, instead of a flat block of paraffine, I employ a roller of that material, made by pouring melted paraffine around a wooden core or axis, placed in a suitable mould. The cloth, which has been previously warmed, is then drawn in a contrary direction to the roller, with which it is kept in very close contact, by suitable pressure.

This plan will serve also for preparing water-proof paper.

The thorough incorporation of the paraffine with the cloth is completed by calendering between hot metallic rollers, as in the previous case.

Sometimes, also, I draw the warmed cloth over a bar, of any suitable form, of paraffine, instead of over

a cylinder of that substance, and then proceed to calender it.

Paraffine can likewise be applied to cloth and leather, by rubbing it on strongly, when cold, and then passing a hot iron over its surface, but the methods previously described, I have found more rapid.

At other times I take solid paraffine, which I heat in suitable vessels, until it is not only melted, but its temperature is raised considerably above its melting-point. A temperature of from 130° to 250° Fahrenheit, is found to answer very well. A plate of iron, or other metal is heated to a temperature considerably above the melting-point of paraffine, and on this plate a sheet of stout paper, or other absorbent material, such as linen, cotton, or woollen cloth, is placed, and evenly coated over with the melted paraffine, by means of a brush or other suitable instrument.

The fabric or leather, which it is wished to impregnate, is then spread out on the paraffine-surface above mentioned, usually with the wrong side of the cloth downward, and if thought desirable, a second paraffined surface is laid upon it, so as to bring the paraffine in contact with both of its sides, and the whole is strongly compressed, by means of a hot flat-iron, or by passing it between hot metallic rollers.

When the impregnation is completed, the material is taken out and allowed to cool.

When fabrics of considerable length have to be treated with paraffine, the process can be made continuous, by passing them over one or more hot wooden or metallic rollers, coated with paraffine from working in a bath of that substance. The excess of paraffine is removed by means of what is called a "gauge-spreader," having a gauger or knife fixed above it, and furnished with screws, so as to regulate the amount of paraffine applied to the roller.

The amount of paraffine can also be regulated by means of a brush, or similar apparatus, also acting on a roller, the thorough incorporation of the paraffine and fabric being subsequently completed with hot rollers, by means of which any excess of paraffine can also be removed.

The quantities of paraffine which are applied to fabrics, and the temperature to which I expose them, vary exceedingly, according to their nature, that is to say, according to the thickness of the fabric, and the delicacy of the colors, as any practical man will readily understand.

I would here remark, that as paraffine has a tendency to crystallize, and thereby detract from the impervious character of the saturated fabric, I find it desirable to mix with it, before applying it to the leather or textile fabric, from five to thirty per cent.

of drying-oil, such as linseed-oil, or nut or poppy-oil, melting the paraffine to facilitate the admixture, and then casting the same in blocks, which are used in the manner above described, or the fabric saturated with the paraffine may have a coating of drying-oil.

My object in applying paraffine to wood, is to fit it the better for being manufactured into vessels of capacity, as vats, cisterns, and casks, or barrels.

The paraffine may be applied to the wood in the form of planks or of staves, or to the vessels when manufactured.

Casks or barrels, for containing ale or beer, may be beneficially treated with pure paraffine. The casks are first to be dried, by hot air, and the melted paraffine is to be poured therein. The casks being then closed, are rolled over and over, until thoroughly saturated. After this, they are to be again heated, and any excess of paraffine contained therein is to be turned out.

*Claim.*

What I claim as my invention, and desire to secure by Letters Patent, is—

The employment and application of paraffine, in a solid state, to wood, leather, paper, or textile fabrics, composed of cotton, linen, wool, or silk, by means of a metal plate, heated to a temperature from 130° to 250° Fahrenheit, the article to be treated to be stretched thereon, and then manipulated, substantially as and for the purpose set forth.

In testimony whereof, I have signed my name to this specification, in the presence of two subscribing witnesses.

Witnesses:

J. HENRY JOHNSON,

47 Lincoln's Inn Fields, London.

HENRY STEVENS,

Clerk to Mr. J. Henry Johnson,

47 Lincoln's Inn Fields, London.